

Aug. 28, 1928.

1,682,590

A. O. AUSTIN

INSULATOR PIN AND PROCESS OF MANUFACTURING THE SAME

Original Filed March 1, 1923



Inventor:

Arthur O. Austin  
By Nissen & Crane  
Atty.

## UNITED STATES PATENT OFFICE.

ARTHUR O. AUSTIN, OF BARBERTON, OHIO, ASSIGNOR, BY MESNE ASSIGNMENTS, TO THE OHIO BRASS COMPANY, OF MANSFIELD, OHIO, A CORPORATION OF NEW JERSEY.

## INSULATOR PIN AND PROCESS OF MANUFACTURING THE SAME.

Original application filed March 1, 1928, Serial No. 621,966. Divided and this application filed October 22, 1925. Serial No. 64,261.

This invention relates to a process of manufacturing insulator pins in which the pin is provided with an insulator supporting tip of soft metal such as lead.

5 The object of the invention is to provide an improved process for securing the tip to the pin, which shall be more reliable in its operation than methods heretofore used, and which shall provide a better union between the pin and its tip.

10 The invention is exemplified by the combination and arrangement of parts and by the steps of process described in the following specification and illustrated in the accompanying drawing and it is more particularly pointed out in the appended claims.

15 The present application is a division of my prior application Serial No. 621,966, filed March 1, 1928.

20 In the drawing the figure is a sectional view of an insulator pin tip having the invention applied thereto.

25 While this invention has especial advantages as applied to insulator pins, it will be understood that certain features of the invention, as pointed out in the appended claims, are of general application and I do not, therefore, wish to restrict the application of the invention to any particular article except as pointed out in the claims.

30 While lead tipped pins have been used in a number of instances, it frequently happens that there is difficulty owing to the lead flowing or becoming loose on the main body of the pin. In order to eliminate the difficulties experienced in ordinary lead-tipped pins the improved method embodying the present application has been adopted. The main body portion 10 of the pin, made of 35 steel or other suitable material, is first galvanized. After galvanizing, the end of the pin which is to be covered by the lead tip is placed in a suitable flux such as zinc chloride or hydrochloric acid. If the flux contains water it is allowed to dry so that it will not cause serious spattering when placed in the lead. The tip of the pin is then

placed in a molten lead bath, where the flux permits amalgamation between the zinc and the lead. At the same time that the amalgamation is taking place the tip of the pin is heated so that the lead will become permanently attached to the same when the pin is placed in the die and molten lead cast around the end, this being done while the pin is still heated from its immersion in the lead bath. The preliminary lead coating and the molded lead cover are shown somewhat diagrammatically and appropriately labeled in the drawing. In addition to the amalgamation the pin is usually roughened or grooved, which affords more surface and a better grip between the lead and the body of the pin. The roughening may also be done in such a way as to increase the effective size of the pin, thereby giving the lead much better support. This is of great advantage where high loads are to be applied or carried by the pin.

35 Another method of securing the desired result is to tin the tip or end with tin or a compound which will melt readily and amalgamate with the lead when the same is cast on the pin. This method insures a bond between the lead or tip and the body of the pin so that the same will not become loose, and permits the pin being used on higher mechanical loads. In some cases a blank only is cast on the tip of the pin and a thread cut or pressed in the same.

40 The melting temperature of lead from which the molded tip may be formed is 328° C. While that of tin is 321° C. and that of zinc with which the pin is galvanized is 419° C. The preliminary coating given the galvanized tin in the presence of a flux is formed of a metal, the melting point of which is no higher than that of the molded tip. This insures complete union of this coating with the molded tip which could 45 not be so readily or surely effective if the tip were molded directly on the pin.

I claim:

1. The process of manufacturing insulator

pins wherein the portion of said pin to which the insulator is to be secured is subjected to a flux and coated with a relatively thin coat of metal, after which a thimble of relatively soft metal is formed upon said coated portion.

2. The process of manufacturing an insulator support wherein a galvanized pin is subjected to a fluxing material and dipped 10 into molten lead to impart a thin coating of lead thereto, after which a thimble of lead is molded onto said coated portion.

3. The process of manufacturing an insulator support wherein a galvanized pin is subjected to zinc chloride to provide a flux, 15 after which the portion of said pin having said flux thereon is dipped into a molten metal to impart a thin coating of metal thereto, and a thimble of soft metal is molded about said coated portion while said pin is still heated.

4. The process of manufacturing an article having a coating of soft metal wherein a metal body is given a coating of metal differing from the material of said body, and thereafter a covering of a third metal is applied to said body over said coating.

5. The process of manufacturing an article wherein a ferrous body member is first galvanized and thereafter a layer of lead applied to the galvanized body.

6. The process of manufacturing a metal article wherein a ferrous body is galvanized, the galvanized body being then dipped into 25 molten lead, and thereafter a layer of lead molded over the coating of lead produced by said dipping.

7. The process of manufacturing a metal article wherein a ferrous body member is galvanized, after which flux is applied thereto and the article dipped in a bath of molten metal, after which a lead covering is molded 40 on said member while said member is still heated from the immersion in said molten metal.

8. A galvanized pin having a portion thereof coated with a metal which has a relatively low melting point and having a covering disposed about said coated part 45 this being of metal having a melting point at least as high as that of the coating.

9. The process of manufacturing an insulator pin, comprising the steps of coating a portion of the pin with a metal having 55 a lower melting point than that of the pin, and thereafter forming a layer of metal over said coating, the metal of said layer having a melting point at least as high as the melting point of said coating.

10. The process of manufacturing an insulator support with a thimble of relatively soft metal, comprising the steps of subjecting a portion of the pin to a fluxing material, then dipping the fluxed portion in a

bath of molten metal, the melting point of 65 which does not exceed that of the metal of which the thimble is composed, and then molding upon said coated portion a thimble of relatively soft metal.

11. The process of manufacturing insulator pins provided with a lead thimble, comprising the steps of fluxing a portion 70 of the pin, then dipping the fluxed portion in a bath of molten metal, the melting point of which does not exceed that of lead, and 75 then molding a thimble of lead onto the coated portion.

12. The process of applying a lead thimble to a galvanized insulator support, comprising the steps of subjecting a portion of 80 the pin to a fluxing material, then dipping the fluxed portion in a bath of molten metal which has a melting point not exceeding that of lead to impart a thin coating thereto, and then molding a thimble of lead upon 85 said coated portion.

13. The process of manufacturing an insulator pin, comprising the steps of galvanizing a ferrous pin body, applying a fluxing material to a portion of the galvanized body, dipping said portion in a molten metal having a melting point lower than the melting point of zinc to apply a coating of said metal to said portion, and thereafter molding a covering of soft metal upon said 95 coated portion, the metal used for said covering having a melting point at least as high as the melting point of the metal used for said coating.

14. An insulator support having a portion 100 thereof coated with metal, the melting point of which is lower than that of said support, and a covering of soft metal on said coated portion, the melting point of the soft metal covering being at least as high 105 as that of said coating.

15. An insulator support comprising a galvanized member having a portion thereof covered with a coating of metal, and a layer of metal disposed on said covered portion, the melting point of said layer of metal 110 being at least as high as that of said coating.

16. An insulator pin comprising a galvanized pin body, a lead tip on said pin body, and a thin coating interposed between said lead tip and pin body to insure close union between said tip and body, said coating being formed of a metal having a lower melting point than zinc and one not exceeding 115 that of lead.

17. An insulator pin of ferrous metal and a soft metal tip formed on said pin and alloyed with the metal of said pin forming a continuous molecular union between said 120 pin and tip.

18. An insulator pin of ferrous metal, a soft metal tip formed on said pin and an

intermediate layer of metal interposed between said pin and tip and alloyed with the metal of said pin and tip and forming a continuous molecular union between said pin and tip.

19. An insulator pin of ferrous metal having the outer surface thereof galvanized and a lead tip formed on said pin, the

galvanizing coating of said pin being alloyed with the metal of said pin and tip to form a continuous molecular union between said pin and tip. <sup>10</sup>

In testimony whereof I have signed my name to this specification on this 17th day of October, A. D. 1925.

ARTHUR O. AUSTIN.